

Jan. 8, 1924.

1,480,471

F. D. S. SANDEMAN

TREATMENT OF JUTE AND LIKE FIBROUS MATERIAL

Filed Sept. 12, 1921



By

Inventor

F. D. S. Sandeman  
Day  
Watson, Cort, Moore & Grindle  
Attn: J. S.

Patented Jan. 8, 1924.

1,480,471

## UNITED STATES PATENT OFFICE.

FREDERICK DAVID STEWART SANDEMAN, OF DUNDEE, SCOTLAND, ASSIGNOR TO JUTE INDUSTRIES LIMITED, OF DUNDEE, SCOTLAND, A COMPANY OF GREAT BRITAIN.

### TREATMENT OF JUTE AND LIKE FIBROUS MATERIAL.

Application filed September 12, 1921. Serial No. 500,114.

*To all whom it may concern:*

Be it known that I, FREDERICK DAVID STEWART SANDEMAN, subject of the King of England, and residing at Dundee, in the 5 county of Forfar, Scotland, have invented certain new and useful Improvements in the Treatment of Jute and like Fibrous Material, of which the following is a specification.

10 This invention relates to the treatment of jute and like fibrous material having long fibres and has for its object to enable the earlier stages in the treatment to which the material is normally subjected to be simplified and a saving of labour to be effected while at the same time a more even sliver is produced.

In the case of jute when this material is removed from the bale and after opening 20 it is commonly subjected to treatment in a softener and subsequently in a breaker card whence the jute comes as a sliver which is dealt with by other processes not pertinent to the present invention. The fibres of the 25 jute when taken from the bale vary in length from about 4 to about 14 feet and owing to this considerable length it is necessary in the process ordinarily employed to utilize hand labour to a considerable extent in the 30 feeding of the material into the softener, in removing it from the softener and subsequently in feeding it into the breaker card. According to the usual procedure the jute as it is taken from the bale is passed 35 through the opener and it is then divided up by hand into "strikes" which are fed by hand into the softener the strikes being manipulated by hand so as to facilitate the 40 passage of the material through the softener. On emerging from the softener the jute is taken by hand and twisted and placed on a barrow where it remains for some hours. Subsequently the jute is placed by hand on the feed sheet of the breaker card 45 in such a way that the fibres will enter this machine in the proper manner.

According to this invention the material after passing through the opener is cut in order to reduce the fibres to a length not 50 exceeding 2 feet and the cut fibres are fed automatically by means of a hopper feed apparatus into the softener. On leaving the softener after remaining the requisite time in the barrow or equivalent the fibres 55 are fed by another hopper feed apparatus

into the breaker card. In the case of jute, for example, when removed from the bale the material is passed through the opener and the fibers are then passed through a machine whereby they are cut into lengths of 60 the desired dimensions. The length of the cut fibres is preferably not less than 7 or 8 inches and may conveniently be in the neighbourhood of 16 inches but the length 65 may be determined by the setting or structure of the carding machines which have to deal with the material and by the nature of the yarn that is to be made. The fibres pass through the cutting machines on a 70 series of band conveyors which carry them away from the machine after cutting and a sorting of the cut fibres may then be effected such sorting being carried out if desired partly or wholly by hand or partly or 75 wholly mechanically. The cut fibres are delivered by a conveyor into a hopper feed apparatus constructed with respect to its general features on known lines. This hopper feed has a certain carding or like effect 80 on the fibres and delivers them somewhat in the form of a blanket to the softener. The fibres travel through the softener and emerge on to a conveyor which delivers the material into barrows in which it lies for 85 the necessary interval. Subsequently the fibres are fed by hand into a second hopper feed apparatus and the blanket of fibres which issues therefrom passes on to the feed sheet of the breaker card which deals 90 with the fibres in the usual manner and delivers the sliver which is subsequently treated in the ordinary way.

The cutting of the fibrous material into relatively short lengths is advantageous 95 from the point of view of the final product and with respect to the earlier steps in the treatment of the material besides effecting an economy in labour. In the first place the sorting that now becomes possible as 100 the fibres issue from the cutting machine enables the material to be graded so that in the case of jute the ends of the fibres can be separated from the central portions which are of better quality and different 105 qualities of material thus separated can be dealt with subsequently in separate machines for the production of different grades of yarn. The passage of the fibres from the cutting machine to the hopper feed may be 110 effected automatically by means of convey-

ers. By reason of the action of the hopper feed apparatus the fibres are formed into a blanket which can be delivered automatically to the softener so that the feeding by hand of the softener is avoided. Owing to the manner in which the hopper feed has dealt with the cut fibres, a more satisfactory softening of the fibres is effected since the liquid delivered on to the fibres as they pass through the softener can take effect on the fibres more thoroughly and readily than when they are in greater lengths when they could not be passed through the hopper feed. Again, as the fibres pass through the softener they can be delivered automatically by a conveyer into the barrows and handling of the material is again avoided or minimized. By employing a hopper feed for delivering the material after it has been removed from the barrows to the breaker card labour is saved and a more even feeding into the breaker card is effected. The fibres can be delivered in bulk to the hopper feed whence a relatively even blanket of fibres flows on to the feed sheet of the breaker card and as a result a more even distribution of the fibres on the feed sheet is obtained and consequently the sliver issuing from the breaker card is more uniform in its density.

A further advantage in the improved method of treating the fibres is that by cutting them so as to reduce their length it becomes possible to employ an automatic feeding mechanism and in addition to getting a more even delivery through the breaker card as mentioned above, this machine has to do less breaking of the fibre and can therefore have a greater carding effect than is possible where fibres of full length are delivered into the breaker card. The fibres in the sliver leaving the breaker card tend to have a greater average length than is the case where the whole reduction in length of the fibres has to be performed in the breaker card.

The accompanying drawing illustrates somewhat diagrammatically and in sectional elevation one arrangement of the apparatus necessary for carrying out the improved process.

The fibres are fed in the ordinary way into the opener A so that they will pass in the direction of their length through this machine. On emerging from the opener it is necessary to transfer the fibres by hand on to the entering table of the cutter B. The slabs of jute as they come out of the opener A are separated by hand into heads and the individual heads of jute are laid across the table or entering ends B' of the conveyer bands of the cutter B and so that the fibres extend transversely across this machine. The fibres are carried through the cutter B and are thereby cut up into lengths not

exceeding two feet. On emerging from the cutter B the short lengths of fibre are delivered by the conveyer bands of the cutting machine into the hopper feed C. The delivery of the fibres may be as shown in the drawing direct from the cutter B into the hopper C or the fibres may pass off the band conveyers of the cutter on to other band conveyers serving to deliver the fibres into several hoppers similar to C. Such an arrangement is usually preferable since the supply of fibres issuing from a single cutting machine such as B is sufficient to feed two or more hoppers. If a sorting of the fibres is to be effected, it is carried out at this stage. For example the length of the delivery end of the cutting machine may be such that as the cut fibres pass out from the cutter on the several conveyer bands a hand sorting can be effected. Thus the end portions of the fibres can be removed and taken away by suitably arranged conveyer bands or by other means so as to enable these portions of the fibres to be dealt with separately while the main part of the fibres pass on into the hopper feed mechanism. In some cases the sorting may be carried out mechanically by arranging for the outer conveyer bands of the cutter B on which will lie the ends of the fibres to deliver these parts of the fibres on to one conveyer band at the end of the machine while the other cut portions of the fibres are delivered either directly into a hopper feed or on to one or more conveyer bands which supply several hopper feed mechanisms.

Each hopper feed apparatus is conveniently constructed and arranged somewhat as illustrated diagrammatically in the drawing with a lattice C' and a stripper C''. As the cut fibres pass through the hopper feed C they are so treated that they issue in substantially blanket form. This blanket of fibres is delivered to the softener D. The fibres fall on to a conveyer or feed sheet D' which carries them to the rollers of the softener D. Owing to the relatively short fibres being in blanket form, they will be carried satisfactorily through the softener and will be prevented from falling down between the rollers of this machine. At the delivery end of the softener the fibres are delivered by a conveyer such as E into the usual barrows F in which the fibres are allowed to lie in the customary manner for a certain number of hours.

When the softening is completed, the fibres are taken by hand from the barrows F and fed into a second hopper feed apparatus G. The fibres as they issue from this hopper are delivered to the breaker card H. As the fibres pass out from the hopper feed G in blanket form they flow on to the feed sheet H' of the breaker card and a uniform feed to the breaker card is thus obtained.

The breaker card H is of usual construction but may be modified in respect of the positions of the stripping rollers in accordance with requirements and the length into which

5 the fibres have been cut in the cutter B.

Each hopper feed mechanism C and G may be constructed as found desirable and in accordance with the length into which the fibres have been cut the machine being

10 arranged so as to pick up the fibres from the hopper into which they are first fed and deliver these fibres in a substantially uniform stream or sheet. A certain carding effect is obtained in the hopper feed whereby the 15 fibres are caused to issue as mentioned in substantially blanket form.

The details of the mechanisms employed in carrying the process into practice may be modified as found desirable more especially 20 in accordance with the length into which the fibres are cut.

What I claim as my invention and desire to secure by Letters Patent is:—

1. A process for the treatment of fibrous material such as jute having long fibres according to which the material is first opened, next the fibres are cut so as to reduce them to a length of from seven inches to two feet. the cut fibres being then passed into a hopper feed mechanism and delivered automatically 25 from therefrom in substantially blanket form to a softener, the fibres after softening being placed in a hopper feed mechanism and delivered thereby to a breaker card.

35 2. A process for the treatment of fibrous material such as jute having long fibres according to which the material is first opened, next the fibres are cut so as to reduce them to a length of from seven inches to two feet, the cut fibres being then passed into a hopper feed mechanism and thereby delivered to a softener, the fibres after softening being placed in a hopper feed mechanism and automatically 40 delivered thereby in substantially blanket form on to the feed sheet of a breaker card.

45 3. A process for the treatment of fibrous material such as jute having long fibres according to which the material is first opened, next the fibres are cut so as to reduce them to a length of from seven inches to two feet, the cut fibres being delivered automatically 50 into a hopper feed mechanism and thereby delivered to a softener, the fibres next being

delivered automatically from the softener 55 into barrows whence the fibres are taken and placed in a hopper feed mechanism which delivers them automatically on to the feed sheet of a breaker card.

4. A process for the treatment of fibrous 60 material such as jute having long fibres according to which the material is first opened, next the fibres are cut so as to reduce them to a length of from seven inches to two feet, the cut fibres being then delivered automatically 65 into a hopper feed mechanism and delivered automatically therefrom in substantially blanket form to a softener, the fibres after softening being placed in a hopper feed mechanism and delivered automatically 70 thereby in substantially blanket form on to the feed sheet of a breaker card.

5. The method of treating long fiber jute preparatory to yarn making consisting in opening the fibres, cutting them into sections 75 having lengths of between seven inches and two feet, forming these sections into a substantially continuous blanket, and feeding the blanket thus formed through a softening machine.

6. The method of treating long fiber jute preparatory to yarn making consisting in opening the fibers, cutting them into sections from seven inches to two feet in length, forming the short lengths into a substantially continuous blanket, feeding the blanket thus formed through a softening machine, forming a second continuous blanket 85 of the softened fibers, and feeding this second blanket through a breaker card. 80

7. The method of treating long fiber jute preparatory to yarn making consisting in opening the fibers, cutting them into sections from seven inches to two feet in length, softening the sections thus formed, 95 forming a continuous blanket of the softened fibers and feeding this second blanket through a breaker card.

8. The method of treating long fiber jute in yarn making consisting in opening the 100 fibers, cutting them into sections from seven inches to two feet in length, softening the sections thus formed, and then carding the same in a breaker card.

In testimony whereof I have signed my 105 name to this specification.

FRED. D. STEWART SANDEMAN.